

[54] **TRIDIMENSIONAL FIBER  
REINFORCEMENT OF PORTLAND  
CEMENT CONCRETE MATRICES**

[75] Inventor: **Antoine E. Naaman, Cambridge, Mass.**

[73] Assignee: **Massachusetts Institute of Technology, Cambridge, Mass.**

[22] Filed: **Aug. 24, 1972**

[21] Appl. No.: **283,438**

[52] U.S. Cl. .... **52/664, 52/600, 52/659,**  
52/736

[51] Int. Cl. .... **E04c 5/01**

[58] Field of Search .... **52/600, 664, 630, 719,**  
52/736, 660, 414, 735, 676, 454, 740, 733,  
734; 245/2, 5

[56] **References Cited**

UNITED STATES PATENTS

|           |         |                      |          |
|-----------|---------|----------------------|----------|
| 906,479   | 12/1908 | Whitacre .....       | 52/733   |
| 1,046,913 | 12/1912 | Weakley .....        | 52/736 X |
| 1,124,170 | 1/1915  | Rechnitz .....       | 52/676   |
| 2,754,674 | 7/1956  | Mulsbury et al. .... | 52/734 X |

Primary Examiner—Henry C. Sutherland

Assistant Examiner—Carl D. Friedman

Attorney, Agent, or Firm—Arthur A. Smith, Jr.;  
Martin M. Santa; Robert Shaw

[57] **ABSTRACT**

Steel fibers or cloth made therefrom having a tridimensional configuration for use as a reinforcement for Portland cement concrete matrices is described. At least three wires, approximately equally laterally spaced from each other, skeletally enclose a volume in the approximate shape of a sphere or ellipsoid; the wires are joined to one another where they meet along the axis of the volume enclosed to form the basic tridimensional element termed an "enclosure". These enclosures may be connected in series by causing the wires to be sufficiently long to form two or more enclosures. One or more of serially connected enclosures may be used as a reinforcing fiber. A continuous fiber is formed by connecting in series a relatively large number of enclosures. A group of parallel, continuous fibers may be laterally connected to form a tridimensional cloth.

**6 Claims, 19 Drawing Figures**



PATENTED DEC 10 1974

3,852,930

SHEET 1 OF 12



FIG. 1



FIG. 2



FIG. 3(A)



FIG. 3(B)



FIG. 3(C)



FIG. 4(A)



FIG. 4 (B)



FIG. 5



FIG. 6



FIG. 7

SHEET 06 OF 12



FIG. 8

SHEET 07 OF 12





FIG. 10

PATENTED DEC 10 1974

3,852,930

SHEET 09 OF 12



FIG. 1



FIG. 12



FIG. 13

PATENTED DEC 10 1974

3,852,930

SHEET 12 OF 12



FIG. 14

## TRIDIMENSIONAL FIBER REINFORCEMENT OF PORTLAND CEMENT CONCRETE MATRICES

This invention herein described was made in the course of a contract, No. DAHC 15-67-C-0222, with the Advanced Research Projects Agency.

This invention relates to a fiber configuration for use as a reinforcement for a concrete matrix and in particular to steel fibers having a tridimensional structure for use as reinforcement in a concrete or cement matrix.

In contrast with fiberglass-plastic composites, where the fibers occupy up to 80 percent of the total volume of the material, steel fibers in a concrete matrix generally occupy no more than 3 percent by volume. Tensile and flexural strength of the concrete is approximately doubled by this low percent of fiber volume. Compressive strength follows the same trend. However, the efficiency of random fiber reinforcement is much less than that of conventional reinforcing steel due to its random orientation and the dispersion in the matrix and also due to discontinuity. Its use in structural elements, when design justifies economical considerations, is mainly in combination with conventional reinforcement.

Steel fibers which are conventionally used have diameters ranging from 4 to 30 mils, a length between onequarter and 2 inches and a tensile strength between 100,000 and 400,000 psi. Obtaining a uniform dispersion of the fibers and preventing their segregation appears to be the most difficult problem in preparing a composite of these fibers and concrete. Experience with steel fibers has shown that segregation is related to two reinforcement parameters: the aspect ratio of the fibers and their fraction volume in the mix. Increasing the aspect ratio or increasing the fraction volume of the fibers increases tendency to segregation and destroys the uniformity of the composite.

The use of steel fibers in concrete is mainly limited by the cost/efficiency ratio. The price per pound of steel fibers will likely remain at least three or four times the cost of conventional reinforcing steel. It seems, therefore, that steel fiber reinforcement in its previous form is not able to compete in applications where conventional reinforcement is satisfactory.

These prior-art fibers have as their primary function that of being an impact or shock energy absorber. However, a second but not less important function for fibers would be as a tensile bearing component identical to conventional reinforcement in reinforced concrete. Experimental data shows that a common description of the failure mechanism of a composite is that, after cracking of the matrix, specimens failed by pulling out of the fibers bridging the fracture surfaces. There exists a lack of bonding leading to a low failure strength. The strength of the fiber is inefficiently used. Attempts to improve this bonding by increasing the length of the fibers results in increasing the aspect ratio which leads to segregation and not the desired composite material. Coating the fibers and improving mechanical bonding by spiralling the fibers or deforming the fibers assist in improving the performance of the composite but are unable to solve the problem completely. Some improvement is expected by using closed form fibers such as rings or rectangles; however, segregation remains a problem.

The tridimensional fibers of this invention can be used as discontinuous reinforcement, as straight fibers are, where the number of basic elements which are serially connected is small and forms a fiber which is not long relative to its lateral dimensions. Such fibers can be mixed with the concrete matrix prior to pouring, incurring less segregation problems than straight fibers. If mixing the discontinuous fibers in the matrix is not desired, the concrete matrix may be poured over the fibers which are previously placed in a form, and pile up due to their tridimensional shape to occupy part or the entire volume of the form. Discontinuous tridimensional fibers are more efficient than straight wires with respect to improvement in tensile strength, toughness, cracking, bonding and ductility.

The tridimensional fibers may also be constructed to form a continuous fiber by serially connecting a group of basic elements whose total length extends over a substantial portion of the length of the structure of which it is to form the reinforcement. These continuous fibers may be formed into a cloth by spaced wires laterally joining parallel spaced continuous fibers. Continuous or cloth tridimensional fibers allow the use of high strength steel while still achieving ductility through crushing of the concrete matrix in which they are embedded when the applied load is high enough. There is also an increase in the efficiency of energy absorption, impact resistance, cracking and ductility. Where cloth is used, there is no need for spacers to laterally and/or vertically separate the continuous fibers.

Tridimensional fibers of the continuous or discontinuous type offer savings in time and labor over conventional reinforcing rods which must be secured in place.

Tridimensional fibers also have the advantage over conventional reinforcing steel that with a relatively simple, inexpensive machine they can be fabricated on-site from spools of wire.

It is therefore an object of this invention to produce a fiber configuration which incurs less segregation problems than prior art fibers if mixed with a concrete matrix prior to pouring or which may, if desired, be placed in a mold prior to pouring the concrete over the fibers.

It is a further object of the invention to produce a fiber which gives the matrix in which it is placed greater tensile strength, bonding, toughening and ductility than obtainable with prior art fibers.

It is a still further object of the invention to produce a fiber which is self-spacing, susceptible to on-site fabrication and capable of being formed as a cloth.

Other objects and features of the present invention will be apparent from the following description of tridimensional fiber elements read in conjunction with figures in which

FIG. 1 shows one embodiment of the tridimensional fiber element, identified as the type 1 element;

FIG. 2 shows an alternate embodiment of the tridimensional element, identified as the type 2 element;

FIG. 3(a) shows a first mode of reinforcing concrete where the tridimensional elements are uniformly disposed;

FIG. 3(b) shows a second mode of reinforcing concrete where tridimensional elements are concentrated in the tensile stress area of the concrete;

FIG. 3(c) shows a third mode or reinforcing concrete where the tridimensional elements are in a single layer just covered by the concrete;

FIG. 4(a) is a graph of stress versus strain for a low yield strength ductile steel fiber;

FIG. 4(b) is a graph of stress versus strain for a high yield strength brittle steel fiber;

FIG. 5 is a graph of load versus elongation for conventional fiber-reinforced concrete under tensile loading;

FIG. 6 shows graphs of load versus deflection for conventional fiber-reinforced concrete under flexural loading;

FIG. 7 shows graphs of load versus deflection for a type 1 tridimensional fiber element reinforced concrete using the first mode of reinforcement with ductile steel;

FIG. 8 is a graph of load versus deflection for a type 1 tridimensional fiber element-reinforced concrete using the second mode of reinforcement with ductile steel;

FIG. 9(a), (b) and (c) are graphs of load versus elongation for a type 1 tridimensional fiber element-reinforced concrete using the third mode of reinforcement with different wire diameters and volume fraction of ductile steel;

FIG. 10 are graphs of load versus deflection of a type 2 tridimensional fiber element-reinforced concrete using the first mode of reinforcement with ductile steel;

FIG. 11 shows graphs of load versus deflection for a type 2 continuous tridimensional fiber element-reinforced concrete using the second mode of reinforcement with ductile steel;

FIG. 12 shows graphs of load versus deflection for a type 2 continuous tridimensional fiber element-reinforced concrete using the second mode of reinforcement with brittle steel;

FIG. 13 shows a graph of load versus deflection for a type 2 continuous tridimensional fiber element-reinforced concrete using the second mode of reinforcement with brittle steel and incompletely cured concrete; and

FIG. 14 shows continuous fibers attached to each other to form a cloth.

The tridimensional fiber of the skeletal type has the property that the bond strength of the steel in concrete is increased by a fiber of this form by adding a mechanical component to bond. Tridimensional fibers may have a great variety of shapes, for instance, that of a tetrapode or spherical skeleton. Two preferred embodiments are shown in FIGS. 1 and 2, where the skeletal arrangement of the wires approximate an ellipsoid. FIG. 1 shows four wires 10 equally spaced from each other to form the skeletal outline 11 of an ellipsoid. The wires are twisted together at the ends 12, 13 of the ellipsoid; and, in the embodiments shown in FIGS. 1 and 2, the wires are continued to form another element 14 identical to that of element 11. Together, elements 11 and 14 form a fiber designated as type 1 fiber in the test results to be subsequently presented.

An alternate embodiment of the tridimensional element is shown in FIG. 2, where only three equally spaced wires 20 form the ellipsoidal skeleton, and the fourth wire 21 joins the others where they are twisted together at the ends 12, 13 of the ellipsoid to form an element 22. Elements 22 and 23 are joined to each

other to form a type 2 fiber as designated in the test results to be subsequently presented.

It is apparent that tridimensional fibers may be fabricated of as little as one of the elements 11 or 22 or may be formed of a large number of serially connected elements. In this application, test results are disclosed for fibers having two elements which have been designated as discontinuous fibers and for fibers having eight elements, which have been designated as continuous fibers.

The type 1 and 2 elements used to perform the tests disclosed in this application had typical respective dimensions  $a \approx 3.2$  to  $3.5$  inches and  $3$  inches,  $b \approx 1$  inch and  $0.75$  inches and  $c \approx 0.5$  inches, where  $a$ ,  $b$  and  $c$  are the dimensions illustrated on FIGS. 1 and 2. To ascertain the effect of wire diameter on the strength of the concrete matrix in which the elements were embedded, wire diameters ranging from  $0.012$  to  $0.032$  inches were used. The wire size for each element tested is given on the figures. Larger wire sizes than those used appear desirable but were not tested because the machine used in fabricating the elements was incapable of handling larger wire sizes.

Besides the higher bonding properties of three dimensional fiber elements in comparison to the ordinary steel fiber, a second advantage is that the fibers may be thrown into a mold before pouring in the concrete matrix because the elements pile up to occupy a volume into which the concrete matrix may penetrate. The concrete matrix may have aggregate limited in size to the openings of the element, and penetration into the element may be assisted by conventional vibration techniques. Therefore, there is considerable freedom in designing the mix, and the risk of segregation is eliminated.

A third advantage of the three dimensional fiber elements relates to their volume-enclosing shape which, upon high enough elongation stresses, tends to cause crushing of the enclosed matrix, which produces a ductile type of failure even though the fibers themselves may be brittle steel of high yield strength. Also, three dimensional fibers act as crack arrestors and toughening agents because of the enormous lateral bonded area they offer the surrounding matrix.

Variations in the shape of the links and the methods of joining the wires along the fiber axis between links are left to the choice of the designer. For example, joining may be obtained by twisting as in preferred embodiments, or by clamping, welding, gluing, etc. Twisting the wires is expected to provide a lower apparent modulus and higher elongations (by untwisting) but should be done uniformly as otherwise the strength of the twisted strand formed would be drastically reduced.

Three methods of using the fiber elements of FIGS. 1 and 2 have been investigated and are presented schematically in FIG. 3. Mode 2 shown in FIG. 3(b) is in some way similar to conventional reinforcement: throwing in a certain amount of fibers which, when ultimately embedded in the matrix, will form the tensile load carrying element. This procedure is very easy, for example, in simply supported beams where reinforcement is needed in the bottom region.

Mode 1 shown in FIG. 3(a) provides the isotropic crack arresting mechanism and toughening effect of conventional fiber reinforced concrete throughout the member being reinforced. Mode 3 of FIG. 3(c) is useful for relatively thin elements where reinforcing action is

needed near both faces and for which fibers may be especially shaped. Slabs, wall panels, shells and pavements are typical applications. This mode may also be attractive for prestressed pavement by means of expansive cements because tridimensional steel fiber may create a very effective triaxial restraint necessary to the prestressing action. In general, what is true for tridimensional fibers holds similarly for strand or cloth made of three dimensional fibers.

The tridimensional fiber has the advantage that the element is well anchored to the concrete matrix by the skeletal shape of the fibers. Transfer of load from fiber to fiber is obtained by shearing of the matrix in between overlapping links. On the other hand, if used as a continuous reinforcement, it has the advantage of increasing the bond strength and efficiency of reinforcement against cracking.

If the applied load is high enough, failure can occur through one or a combination of the following situations: (a) the fibers, if discontinuous, pull out; but, due to their bonding properties, this occurs at a much higher load than with straight fibers, everything else being equal; (b) the wires forming the fiber reach their yielding point and lead to the failure of the member; (c) the matrix volume, sustaining the load transfer between overlapping discontinuous fibers, reaches its failure point; (d) the matrix inside the volume enclosed by fiber reaches its failure point under complex multiaxial stresses.

It is a priori easy to imagine that, for a combination of specific variables, ductile failure of a three dimensional fiber-reinforced member may be expected at a relatively high enough stress. For example, for failure as in (b), it is sufficient that the wire be ductile. In the last two cases, (c) and (d), it seems necessary that the load carried by the fiber is higher than some particular value beyond which the matrix will be crushed, allowing further elongation of the fiber and therefore ductility for the member. In other words, a combined action is expected for ductile behavior.

The testing program consists of two major parts: the first one deals with specimens reinforced with straight steel fibers; and, for comparison, the second one uses the two types of tridimensional fibers of FIGS. 1 and 2.

#### Matrix Composition

Essentially the same mortar matrix was used throughout the test program. High early Portland cement type III and fine graded Ottawa silica sand (ASTM C-109) were mixed with water in the following proportions: water to cement ratio = 0.6; sand to cement ratio = 2.5.

For the tests involving tridimensional fibers, the fibers were thrown into the empty mold and then the mortar matrix was poured. A slight vibration was applied to allow good penetration. However, using the straight fibers, the fibers were thoroughly mixed with the mortar matrix before casting. It was observed that the mix becomes more and more stiff with increasing fiber concentration. This is the main reason for which the fraction volume of fibers was kept less or equal to 4 percent, the limit below which the mix is still reasonably workable.

All specimens were poured in plexiglass molds. After 24 hours they were removed from the molds, cured in water at room temperature for 6 days and tested on the

seventh day, except for series G which was tested before curing, i.e., tested 24 hours after pouring.

#### Prior Art Straight Steel Fibers

For purposes of comparison with the tridimensional fiber elements of the invention, tests were made of straight steel fiber reinforced concrete with parameters within average values recommended by most previous investigators in order to avoid experimental obstacles, mainly segregation of the fibers, etc. Typical load elongation curves for tensile and flexural specimens reinforced with straight steel fibers are shown in FIGS. 5 and 6, respectively. The fibers used were high yield, brittle steel, as in FIG. 4(b), 0.75 inches in length and 0.016 inches in diameter, uniformly mixed in the concrete matrix.

The fractional volume of fibers is shown on the curves of the figures. It is seen that higher fractional volumes of fiber produces higher peak load capacity and greater energy absorption which is measured by the area under the load-elongation or load-deflection curves.

#### Tests of Tridimensional Steel Fibers

The second part of the test program consists of several series of single tests under flexural loading, except for series C which was tested under tension. Both types of tridimensional fibers described in FIGS. 1 and 2 were used under the three reinforcing modes indicated in FIG. 3: namely, mode 1 and 2 for flexure, mode 3 for tension.

Two types of steel wires were used for the tridimensional fibers tested in this study: stainless steel with low yield stress and very high ductility, carbon steel with high yield and low ductility. Typical stress elongation curves are illustrated in FIG. 4.

For series A, B and C, tridimensional discontinuous fibers, the type 1 element of FIG. 1 and stainless steel low yield ductile wire were used under the three reinforcing modes already mentioned. Series A, FIG. 7, corresponding to the first reinforcing mode of FIG. 3(a) was made up of three specimens having different volume fractions of fibers (obtained by using different wire diameters). Fibers were thrown into the mold where they piled up filling it completely. Then, the mortar matrix was poured, and a slight vibration applied to insure good penetration.

Series B, FIG. 8, corresponding to the second reinforcing mode of FIG. 3(b), consisted of only one specimen in which the fibers were thrown into the lower half part of the beam in order to form the tensile load carrying element (similarly to conventionally reinforced structures).

Series C, FIG. 9, investigated the third reinforcing mode of FIG. 3(c) by working with tensile plates. One layer of fibers was thrown into the mold, and then just enough mortar was poured to cover it completely. Thickness of the specimen was recorded before testing. The three specimens C1, C2 and C3 of FIGS. 9(a), (b) and (c), respectively, had the following dimensions: 2  $\times$  0.625  $\times$  12, 2  $\times$  0.825  $\times$  12 and 2  $\times$  0.75  $\times$  12 inches.

The series D, FIG. 10, experiments were mainly intended to repeat series A using the FIG. 2 type of tridimensional discontinuous fibers. However, due to difficulties in producing the fibers, smaller wire diameters were chosen.

Series E, FIGS. 11, 12 and G, FIG. 13, were performed in order to investigate the behavior of specimens reinforced with tridimensional continuous fibers

of type 2 elements. Each specimen was reinforced with 20 strands thrown in the lower half of the beam. Series E was divided into two parts using the two types of steel mentioned: low yield, high ductility, FIG. 11, and high yield, low ductility, FIG. 12. Strength and ductility of the reinforced members had to be compared. As the ductility of specimens E3 and E4 (reinforced with high strength strands) was quite low, it was necessary to investigate the mutual interaction between the load carried by the fiber and the matrix. It would have been necessary to use higher diameter wires to investigate the possibility of a ductile type of failure due to a crushing of the matrix within the volume enclosed by the element. As it was difficult, with the available equipment, to produce tridimensional strands of higher diameters, the strength of the matrix was reduced instead. Therefore, specimen G was prepared with the tensile reinforcement as specimen E4 and with the same matrix composition, but was tested 24 hours after pouring, when the strength of the matrix would have been 20 to 30 percent of the expected strength at 7 days. The failure of specimen G was much more ductile than E4 proving that it is possible to obtain ductile failure by a combined interaction between fibers and matrix.

#### Testing Procedure

All testing was performed using an INSTRON Universal testing machine which applied load at a rate of 0.05 inch/minute for all the flexural and tensile tests. Load-deformation curves were automatically plotted on a chart recorder. These deformations, representing deflections or elongations, are the sum of the specimen deformation and that of the testing system. Their value is, therefore, comparative but not absolute. The load deformation curves are shown in FIGS. 5-13.

#### Discontinuous Reinforcement

Considering first series A, B, C and D which involved the use of tridimensional discontinuous fibers of either type 1 or 2 made with ductile steel, FIGS. 7-10, it is observed that higher ultimate stresses, more drastic crack propagation and more significant ductile failure and so energy absorption was obtained than with straight steel fibers as shown in FIGS. 5 and 6. Even at relatively low percentages of reinforcement, the post-cracking load was higher than the first crack load and yield type behavior occurred before failure. The drop in the load-deformation curve after maximum load was in general very smooth, creating a kind of plateau, typical of good ductile behavior and energy absorption. This occurred even for specimen B, which was only partially reinforced as in conventional beams. The number of cracks in the middle of the flexural beams was significantly higher, at least 5, compared to one crack that developed in a similar specimen reinforced with straight fibers. This results from the higher efficiency of tridimensional fibers due to their length, bonding properties, higher directionality and geometrical shape.

Comparing the load curves of FIGS. 7-10 with respect to load and ductility, we can observe better results in series A, reinforced with type 1 fibers, than in series D, reinforced with type 2 fibers. A priori it had been expected, at least with respect to strength, that the type 2 fibers would be better. However, it was observed that, in series D, the main crack occurred and opened along a section where a big number of fiber ends were visible. The presence of a higher concentration of ends in a cross section is due to the end plate effect of the molds. In order to reduce this effect, a V-

shaped piece of wire mesh was placed at each end of the mold in series A, B and C. This procedure was not followed for series D. However, this sort of effect would be automatically eliminated in a member of larger size, or greatly reduced by using discontinuous fibers of different sizes. Results of tensile tests in series C are somehow difficult to compare with those obtained with straight fibers, due mainly to differences in the geometry of the specimens and the testing apparatus used. Qualitatively, however, FIG. 9 shows an improved ductile type of failure for tridimensional fibers as well as high cracking and disruption of the matrix close to the major opening crack.

Comparing FIGS. 6 and 7, we can easily see that the energy absorbed at failure, taken as area under the load deflection curve, in series A (tridimensional fibers) FIG. 7, as an example, is one order of magnitude higher than a similarly reinforced specimen of straight fibers, FIG. 6. This trend is general, as shown in the other series of experiments, FIGS. 8-10. It should be noted, however, that the ductile property of the steel has certainly also considerable influence on the ductile failure observed in these tests.

No shear failure was observed in specimens uniformly reinforced (Mode 1, series A-D) indicating that tridimensional fibers, similar to straight fibers, do enhance the shear resistance of the concrete matrix.

#### Continuous Reinforcement

At failure the tridimensional strand reinforced beams of series E of FIG. 11, 12 and G of FIG. 13 showed extensive crack propagation in the region of the constant moment. In series E, specimens E3 and E4, FIG. 12, reinforced with high yield, brittle steel, showed much lower ductility at failure than specimens E1 and E2, FIG. 11, reinforced with low yield, ductile steel, while a similar order of strength was observed for the same fraction volume of reinforcement, E1 versus E4. These results indicate that the steel properties are of major importance; and that, in this particular series of tests, ductility of the steel leads to a ductile type of failure. In general, failure occurred progressively with the fracture of the reinforcing fibers by one or more of their wire components.

From the results in series E, it is deduced that, for the particular characteristics of the components used, the ductility of the steel determined whether there was ductile behavior of the member before failure. As it was mentioned earlier, specimen G of FIG. 13, having the same tensile reinforcement as E4, was meant to investigate the possibility of a combined action between tridimensional fiber and matrix which will result in a ductile type of failure. This action was obtained by testing specimen G just 24 hours after pouring, at which time the compressive strength of the matrix was relatively low. Under applied tensile stresses the skeletal part of the tridimensional fiber tends to stretch, crushing the inner, weak concrete matrix and so allowing for more extension and ductility. The improvement in ductility can be observed by comparing the load deflection curves of specimens E4 of FIG. 12 and that of FIG. 13.

In summary of the test results, it can be said that, on the basis of strength, tridimensional continuous reinforcement gave, in general, lower values than theoretically predicted using A.C.I. ultimate moment formula for reinforced concrete; while, on the basis of cracking propagation, ductility and energy absorption, drastic

improvements over conventional reinforcement have been achieved.

What is claimed is:

1. A reinforcing fiber for a concrete matrix comprising

a plurality of three or more steel wires, said wires forming a skeletal outline of a volumetric enclosure, said wires being substantially equally spaced from each other on said enclosure, said wires being joined together at opposite ends of the enclosure, an additional steel wire through the center of said volumetric enclosure, joining the other skeletal wires at the ends of the enclosures.

2. The reinforcing fiber of claim 1 comprising, in addition,

a plurality of said fibers, said fibers being serially connected at the ends where said wires are joined together to form a continuous fiber having a plurality of enclosures.

3. The reinforcing fiber of claim 2 wherein said wires forming a fiber enclosure are continued without being broken and formed into serially connected fiber enclosures called a continuous fiber.

5 4. The reinforcing fiber of claim 3 wherein the wires forming the fiber enclosures are twisted about one another in the region between the enclosures and at the ends of the continuous fiber to achieve the enclosures' connections.

10 5. A reinforcing cloth comprising a plurality of continuous fibers as in claim 2 arranged in a parallel relation and spaced from each other,

a plurality of wires substantially parallel and transverse to the direction of said continuous fibers, each wire of said plurality being connected to a continuous fiber to form a grid-like fiber cloth.

15 6. The fiber of claim 2 wherein said joined wires are wires that are twisted about each other.

\* \* \* \* \*

25

30

35

40

45

50

55

60

65